# EUROPEAN PATENT SPECIFICATION

(11) **EP 0 128 644 B1**
(45) Date of publication and mention of the grant of the patent: **16.09.1987**
(21) Application number: 84302486.0
(22) Date of filing: 11.04.1984
(51) Int. Cl.: F28F 11/02, F16L 55/16

(54) **Heat exchanger tube repair**
Reparieren von Wärmetauscherrohren
Réparation de tubes d'échangeur thermique

(30) Priority: 13.04.1983 GB 8309988; 13.05.1983 GB 8313266
(43) Date of publication of application: 19.12.1984
(73) Proprietor: UNITED KINGDOM ATOMIC ENERGY AUTHORITY, London SW1Y 4QP (GB)
(72) Inventor: Roach, Peter Francis, Croft Warrington Cheshire (GB); Duncombe, Edward, Hale Altrincham Cheshire (GB); Hulse, Ian, Warrinton Cheshire (GB); Stacey, John, Breightmet Bolton (GB)
(74) Representative: Collingwood, Anthony Robert (GB)

## Description

This invention relates to the repair of heat exchanger tubes.

There is currently a problem in the nuclear field, and probably in other fields, where a leak at a tube in a nest of tubes where it is welded to a tube plate in a heat exchanger has to be made good without gaining access to the outside of the tube. The practice for dealing with this problem is to insert a length of repair tube into the leaking tube through the tube plate with one (the outer) end of repair tube explosively welded to the tube plate and the other (the inner) end brazed to the leaking tube. This method of repairing the leaking tube is described in GB-A-2032559.

We have now discovered that the quality of the braze can be affected by the presence of strain in the tube being repaired, such strain arising during the heating necessary to effect the braze. A predetermined tolerable level of said strain can be assessed by tests involving the brazing of specimens under various strains and then inspecting the brazes.

The present invention provides a method for the repair of a leaking heat exchanger tube in a nest of tubes welded to a tube plate which the tube is of U-tube shape and/or passes through one or more support grid plates, said method involving the known step of inserting a length of repair tube into the leaking tube with one end of the repair tube brazed to the leaking tube characterised in that compressional strain in the leaking tube is measured whilst heating the tube to the brazing temperature and the brazing is only effected if the strain is below a predetermined level.

The invention also provides apparatus for carrying out the above method, said apparatus being in the form of a probe which can enter along the leaking tube, the probe being provided with a strain gauge head comprising at least one strain gauge of the kind which can be held in contact with and later released from the inside wall of the leaking tube, characterised in that a heating element is provided in the body of the probe for internally heating the tube to the brazing temperature, and the strain gauge head is connected to means for recording the compressional strain that arises during heating of the leaking tube prior to brazing.

Strain, of a magnitude sufficient to impede the brazing process, does not always occur when a tube is heated. When it does it may be due to the fact that the complete heat exchanger tube is "U" shaped and heating one leg will cause a strain, the magnitude of which is dependent on the bend radius. On the other hand, the stress may be caused by the tube binding in the first (top) support grid plate or any of the lower grid plates through which it passes. In either case, the strain produced may be higher than can be tolerated.

To enable the strain to be measured regardless of its cause, the length of the probe apparatus is such that, for a given heat exchanger, the strain gauge head reaches a region close to but just above the first tube support grid plate. For practical reasons, the heater (and heated region) is kept as remote from the strain gauge as possible, the heater extending downwards from just below the tube plate.

The invention will now be described further with reference to the accompanying drawings in which:
Figure 1 is a cross-sectional elevation of a repaired leaky tube, the figure being used for explanatory purposes;
Figure 2 is a cross-sectional elevation of a leaky tube having inserted therein a probe according to the invention in order to carry out a test according to the invention;
Figures 3A-C are diagrams showing various arrangements of a measuring system;
Figure 4 is a diagram illustrating a junction box; and
Figures 5A, 5B and 5C show three stages in treating an overstrained tube.

In Figure 1 a repaired tube 10 is shown. This tube 10 is one of a nest of similar "U" shaped tubes in a heat exchanger having a tube plate 11 and a top tube support grid plate 12. The tube 10-is welded to the tube plate at a weld 13. It is this weld that can leak after the heat exchanger has been used and it is inaccessible for repair because of the close proximity of other tubes in the nest. If the heat exchanger has been in use as a part of a nuclear reactor installation it is probable that the weld is also inaccessible because of nuclear activation.

It is already known to repair a leak arising at weld 13 by inserting a repair tube 14 which is explosively welded to the tube plate at weld 15 (indicated by X's) and brazed to the tube 10 at a braze 16.

However, in carrying out this known repair (which involves a high temperature - red heat - on the tube 10 to effect the braze) a stress can arise in the tube 10 if the tube 10 is not sufficiently free when expanding. This stress is found to affect the quality of the braze 16 and in particular the evenness of the braze is disturbed.

With this discovered, and in accordance with the invention, the tube 10 is subjected to a strain- on-heating test prior to effecting the repair. This is illustrated with reference to Figure 2.

A probe form of apparatus 20 is inserted into the tube 10. The probe has at its nose a strain gauge head 21. The body 22 of the probe extends from the tube plate 11 to a point close to the gauge head 21, space being left for a junction box 30 (see Figure 4) between the body 22 and gauge 21. The body has an electric heater coil 23 and a coil spacer 24. Service connectors to the probe are indicated diagrammatically by the tube 25 and are described in more detail below.

The strain gauge is of the kind disclosed in GB-A-1,395,263. This gauge has a casing 26 and windows 27 at 90° through which strain gauges 28 having abrasive surfaces 29 can be advanced by a pressure internal to the casing 26. The pressure urges the surfaces 29 into non-slip engagement with the tube 10. This action can be performed remotely by air pressure in a line in the services tube 25. Disengagement of the gauges 28 and tube 10 is effected by releasing the air pressure. In this application of the gauge described above, only one strain gauge is used. The second being held as a spare.

In use the tube 10 is heated by the coil 23 and the strains in gauge 28 are monitored. If strain below a predetermined level is registered then the repair shown in Figure 1 can be made.

Reference is made to our earlier EP-A-109798 (published 30.5.84) which discloses apparatus suitable for making said repair.

The probe apparatus 20 will now be described in greater detail with reference to Figures 3A, B and C and Figure 4 of the drawings.

Figure 3 shows various schematic arrangements of the measuring system. When using a strain gauge of the kind disclosed in GB-A--1,395,263, the service lines must pass through the heated zone and must therefore be of a high temperature type (e.g. mineral insulated cable).

A junction box is required to join the flexible, relatively low temperature service lines used on the gauge described in GB-A-1,395,263, to the rigid high temperature lines required. This box is shown in Figure 4.

The gauge head 21 has two two-wire cables 31, 32, (one for each strain gauge) and a plastic tube air line 33.

At the junction box the wires 31a, 31b of cable 31 are connected to mineral insulated thermocouple cable 34. The wires of cable 32 are similarly connected to mineral insulated cable 35. The line 33 is connected to a rigid air tube 36. The cables 34, 35 are both four-wire mineral insulated thermocouple cable having two alumel conductors and two chromel conductors. When the instrument is in use, one of these cables is coupled with a four terminal digital strain indicator 37. The conductors are disposed within the junction box as shown in one or other of Figures 3A-C. The air line 33 has a glass sleeve covering.

The heater element 23 comprises five-start helical coils of swaged heater cable (1 mm) wound round the body 22. The cable has unswaged, thicker tails which pass outside the tube 25. The swaged coils are held in place on the body 22 with tack welded thin stainless-steel plates. The body 22 is penetrated at a point midway along the element 23 to provide a thermocouple junction at the end of a thermocouple cable which passes along the tube 25 and body 22 so that the temperature of the tube 10 can be assessed.

The coil spacers 24 (each of 1.5 mm diameter wire) centralise the heater in the tube 10 and are held in position by thin tack welded plates. Thus spacers can be provided at the end and centre of the body 22. In Figures 3A-C various ways of connecting the strain gauge 21 to a digital strain indicator 37 via a junction box 30 and 4-core mineral insulation cable 34, 34a, 34b are shown. Figure 3A is a quarter bridge arrangement and Figure 3B is a half bridge arrangement. The conductors are marked "Cr" for a chromel conductor and "Al" for an alumel conductor. Figure 3C shows a fully compensated arrangement.

Connections to the spare gauge (via cable 35-Figure 4) are identical.

From time-to-time use of the invention will expose situations in which the strain is such that a braze cannot be made until the strain is relieved. Two ways are now described of effecting strain relief.

When the tube being repaired is of U-shape the principal strain may be caused by the fact that one leg of the U-shape is being heated whilst the other is not. The magnitude of this basic strain tends to be related to the spacing apart of the legs of the U-shape: a wide spacing gives low strain whilst a close spacing gives a higher strain. Such strains can be relieved by executing a heating step on one leg whilst the other leg is also heated. Said other leg may even be given a repair tube so that both legs have equal treatment even though a leak on the other leg does not exist.

Alternatively, the principal strain may be caused by the leaking tube binding in a support grid plate. Such strain can be relieved by creating in the leaking tube, in the region between weld and braze, a weakness zone so that the tube strain relieves itself at that zone when heated.

Problems arise in choosing the best way to create a weakness zone. A weakness created by simple thinning of the tube does not give the required strain relief, neither does cutting nor drilling. Cutting and drilling is also undesirable as it causes loss of back-up containment that the leaking tube provides despite the fact that it has a leak. This loss also arises if the leaking tube is severed.

Preferably the weakness zone is created first by a thinning operation (such as by undercutting) and second by an expansion or bulging operation at the point of thinning. The expansion or bulging can be performed by using an axially compressed recoverable isostatic ring, such as a rubber ring. With such a zone created, strain arising by the heating of the heat exchanger tube relieves itself at least to a degree not affecting the braze.

This approach to strain relief will now be described further with reference to Figures 5A, 5B and 5C.

In Figure 5A, a leaky heat exchanger tube 50 having an external diameter of 25 mm and a wall thickness of 2.5 mm is given an annular undercut 51 to remove 2 mm of wall thickness over a length of 12 mm. Sharp corners 52 are removed and the undercut has rounded corners 53. The undercut is made above the region at which a braze is to be effected between the tube 50 and a repair tube but close enough to experience the heat of the braze.

In Figure 5B a rubber plug 54 is shown subjected to axial compression (arrows 55) so that is expands into the undercut 51 to give the tube 10 a bulge 56 at the undercut.

Figure 5C shows the shape 57 taken by the undercut 51 when the tube 50 yields (arrows 58) 1.5 mm, on being heated due to the fact that the tube 50 is binding in a grid plate. Yield takes places at about 900°C. The braze is effected at about 1000°C. In this way no troublesome axial strain exists in the heat exchanger tube 50 during the course of the braze and hence there is no tendency for the tube 50 to distort under the strain in the region of the braze. Such distorting, if it occurs, is believed to cause unsatisfactory brazing as the capillary gap between the tube 50 and the repair tube becomes irregular and the braze metal does not spread uniformly.

## Claims

1. A method for the repair of a leaking heat exchanger tube in a nest of tubes welded to a tube plate which tube is of U-tube shape and/or passes through one or more support grid plates, said method involving the known step of inserting a length of repair tube into the leaking. tube with one end of the repair tube brazed to the leaking tube characterised in that compressional strain in the leaking tube is measured whilst heating the tube to the brazing temperature and the brazing is only effected if the strain is below a predetermined level.

2. Apparatus for carrying out the method of claim 1, said apparatus being in the form of a probe which can enter along the leaking tube, the probe being provided with a strain gauge head comprising at least one strain gauge of the kind which can be held in contact with and later released from the inside wall of the leaking tube, characterised in that a heating element is provided in the body of the probe for internally heating the tube to the brazing temperature, and the strain gauge head is connected to means for recording the compressional strain that arises during heating of the leaking tube prior to brazing.

3. Apparatus as claimed in claim 2 in conjunction with a leaking tube passing through a support grid plate in which the length of the probe is such that the strain gauge head reaches close to but just above the support grid plate.

4. Apparatus as claimed in claim 2 in which the or each strain gauge has flexible low temperature connectors to a junction box at which connections are made to a rigid air line and four-wire mineral insulated thermocouple cable to a four-terminal strain indicator giving either a quarter bridge, half bridge, or fully compensated arrangement.

5. A method for the repair as claimed in claim 1 in which the leaking tube is of U-shape, including heating both legs of the U-shape so that strain in the leaking tube is relieved.

6. A method of repair as claimed in claim 1 including creating a weakness zone in the leaking tube, prior to effecting the braze, by thinning the tube and bulging it at a region close enough to the braze region for the weakness zone to experience the heat of the braze to allow yield at that zone.

## Patentansprüche

1. Verfahren zur Reparatur eines lecken Wärmeaustauscherrohres in einem Satz von Rohren, die mit einer Rohrplatte verschweißt sind, wobei dieses Rohr U-förmig ist und/oder durch eine oder mehrere Trage-Gitterplatten hindurch verläuft, mit dem bekannten Schritt, einen Längenabschnitt eines Reparaturrohres in das lecke Rohr einzuführen, wobei ein Ende des Reparaturrohres mit dem lecken Rohr hart verlötet wird, dadurch gekennzeichnet, daß die Druckspannung im lekken Rohr gemessen wird, während man das Rohr auf die Löttemperatur erwärmt, und daß der Hartlötvorgang nur dann durchgeführt wird, wenn die Spannung unter einem bestimmten Niveau liegt.

2. Vorrichtung zur Durchführung des Verfahrens nach Anspruch 1, wobei die Vorrichtung die Form einer Sonde aufweist, die längs des lecken Rohres eindringen kann, und die Sonde mit einem Spannungsmeßkopf versehen ist, der mindestens eine Spannungsmeßeinrichtung jener Art aufweist, welche in Berührung mit der Innenwand des lecken Rohres gehalten und später hiervon gelöst werden kann, dadurch gekennzeichnet, daß ein Heizelement im Körper der Sonde vorgesehen ist, um das Rohr von innen her auf die Löttemperatur zu erwärmen, und daß der Spannungsmeßkopf an eine Einrichtung zum Aufzeichnen jener Druckspannung angeschlossen ist, welche während des Erwärmens des lecken Rohres vor dem Löten auftritt.

3. Vorrichtung nach Anspruch 2, in Verbindung mit einem lecken Rohr, das durch eine Trage-Gitterplatte hindurchtritt, wobei die Länge der Sonde so bemessen ist, daß der Spannungsmeßkopf nahe bis zur Trage-Gitterplatte und gerade bis über diese reicht.

4. Vorrichtung nach Anspruch 2, wobei der oder jeder Spannungsmeßfühler flexible Niedertemperaturanschlüsse an einer Anschlußdose hat, an der Verbindungen zu einer starren Freileitung und über ein mineralisoliertes Vier-Draht-Thermoelementkabel zu einer Spannungsanzeigeeinrichtung mit vier Anschlüssen hergestellt sind, die entweder eine Viertelbrückenanordnung, eine Halbbrückenanordnung oder eine voll kompensierte Anordnung liefert.

5. Reparaturverfahren nach Anspruch 1, wobei das lecke Rohr U-förmig ist, mit der Erwärmung beider Schenkel der U-Form, so daß die Spannung im lecken Rohr entlastet wird.

6. Reparaturverfahren nach Anspruch 1, mit der Erzeugung einer schwächezone im lecken Rohr vor dem Ausführen des Lötvorganges dadurch, daß man das Rohr in einem Bereich dünner macht und ausbaucht, der nahe genug am Bereich der Lötung liegt, daß die Schwächungszone die Wärme des Lötvorganges erfährt, um in dieser Zone ein Nachgeben zu ermöglichen.

## Revendications

1. Procédé pour réparer un tube d'échangeur de chaleur qui fuit, dans un faisceau de tube soudés à une plaque tubulaire, ce tube étant en forme de U et/ou traversant une ou plusieurs plaques perforées de support, ledit procédé impliquant l'étape connue consistant à insérer une longueur de tube de réparation dans le tube qui fuit, avec une extrémité du tube de réparation brasée au tube qui fuit, procédé caractérisé en ce qu'on mesure la contrainte de compression s'exerçant dans le tube qui fuit pendant le chauffage du tube à la température de brasage et l'on n'effectue le brasage que si la contrainte est inférieure à un niveau prédéterminé.

2. Appareil pour mettre en oeuvre le procédé de la revendication 1, ledit appareil étant sous la forme d'une sonde qui peut pénétrer dans le tube qui fuit, le long de ce tube, la sonde étant pourvue d'une tête à jauge de contrainte comprenant au moins une jauge de contrainte du genre pouvant être maintenue au contact de la paroi interne du tube qui fuit et pouvant ultérieurement être détachée, de cette paroi, appareil caractérisé en ce qu'un élément chauffant est prévu dans le corps de la sonde, pour chauffer intérieurement le tube à la température de brasage, et en ce que la tête à jauge de contrainte est reliée à des dispositifs destinés à enregistrer la contrainte de compression apparaissant pendant le chauffage du tube qui fuit, avant la brasure.

3. Appareil selon la revendication 2, de concert avec un tube qui fuit traversant une plaque perforée de support, dans lequel la longueur de la sonde est telle que la tête à jauge de contrainte vient très près de la plaque perforée de support, mais se trouve juste au-dessus de cette plaque.

4. Appareil selon la revendication 2, dans lequel la ou chaque jauge de contrainte comporte des connecteurs flexibles, pour service à basse température, de liaison avec une boîte de dérivation à laquelle on effectue des connexions avec un conduit rigide à air, ainsi qu'un câble de thermocouple à isolation minérale et à quatre fils, relié à un indicateur de contrainte à quatre bornes donnant un agencement à quart-de-pont, à demi- pont, ou entièrement compensé ou équilibré.

5. Procédé pour réparer selon la revendication 1, dans lequel le tube qui fuit est en forme de U, comprenant le chauffage des deux branches du U de façon à relâcher ou éliminer la contrainte dans le tube qui fuit.

6. Procédé pour réparer selon la revendication 1, comprenant la création d'une zone de faiblesse dans le tube qui fuit, avant d'effectuer la brasure, en amincissant le tube et en y créant un renflement en une région assez proche de la région de brasage pour que la zone de faiblesse soit soumise à la chaleur du brasage afin de permettre une déformation par affaissement dans cette zone.
